

## UNITED STATES PATENT OFFICE

CLAUDE CLEMENCION, OF CALUIRE-ON-THE-RHONE, FRANCE

PROCESS OF MANUFACTURING CREPES WITH THREADS OF CELLULOSE ACETATE  
ARTIFICIAL SILK

No Drawing. Application filed March 11, 1932, Serial No. 598,308, and in France March 16, 1931.

The present invention has for its object a process of manufacturing crepes with threads of cellulose acetate artificial silk.

The fabrics with crepe effect are obtained 5 by the employment of highly twisted threads (2000 to 3000 turns per metre or more or less, in accordance with the material employed and its titre). These threads are generally provided naturally or artificially 10 with a gum or glue which opposes their untwisting in the course of the operations that they have to undergo up to and including the weaving. They may be employed in the warp or in the weft, separately or together. 15 The fabric obtained is then subjected to a washing operation intended to remove the gum or glue which fixes the twist; in the course of this washing operation, the fabric undergoes a shrinkage in the direction of the 20 hard twisted threads, which is accentuated by the fact that the fibre swells in the washing bath. When the fabric is dry, it presents the characteristic crepe appearance.

In order to obtain this appearance, a certain amount of twist is therefore necessary 25 which is variable with the properties of the material employed. According to the present invention, it has been found that the twist to be applied to threads of cellulose acetate, in order to obtain crepe, must be greater 30 than that which is applied to threads of viscose. The example, if 2000 turns per metre are sufficient for a thread of viscose with a titre of 100 deniers, 2900 to 3000 turns per 35 metre will be necessary for a thread of cellulose acetate of the same titre in order to have a real crepe after the usual treatments called "scouring."

Now, if it is endeavoured to give such 40 twists to such a thread of cellulose acetate, the following results are obtained:

1. Numerous elementary fibres and often the whole of the fibres—i. e., the whole thread—break.
2. The excess of twisting produces small

kinks, points at which the torsion couple has not been exerted around the axis of the thread, but around another different axis.

3. The resistance to breaking is considerably reduced (it falls to one third of its 50 original value and frequently even lower).

4. The breaking elongation is similarly greatly diminished.

A thread having such properties is unusable and as, moreover, such a result could 55 only have been arrived at by permanently elongating the thread, the effect of crepe is not obtained. It is only possible in practice to give a thread of cellulose acetate with a titre of 100 deniers a twist of 2000 to 2200 60 turns per metre, which is insufficient for obtaining by the usual washing treatments called "scouring" the creping of a fabric consisting of these threads.

It has been attempted to obtain the crepe 65 effect by the action of swelling liquids on the fabric. There is obtained in this way a shrinkage comparable with that which is obtained by the mercerization of cotton and not with that of the creping of silk. In fact, in 70 the case of a warp of cellulose acetate which has not been hard twisted, the latter shrinks more than the weft and, by drawing the fabric together, opposes the crepe effect. As a matter of fact, the fabric obtained in this 75 way does not possess the appearance, the feel, the firmness or the elasticity of a crepe.

According to the present invention, it has been found that it was possible to give the threads of cellulose acetate much greater 80 twists when they were subjected to a preliminary treatment which consisted in a physical modification of the thread of cellulose acetate which left its chemical and tinc-torial properties unchanged. This physical 85 modification results from the action of an agent for swelling the cellulose acetate, with or without the addition of a colloid adapted on drying to leave an elastic coating on the thread. The swelling of the cellulose ace- 90

tate, when it reaches amounts that are greater than those obtained with water, causes a permanent physical modification of the fibre. This modification is preserved after the 5 swelling agent has been removed either by drying, if it is sufficiently volatile, or by suitable washings with water or any other suitable liquid, the washings being followed by drying. The thread has then undergone 10 an internal physical modification the most apparent manifestation of which is a shrinkage (diminution in its length) and which is also characterized by the increase in its breaking elongation and by a break in the 15 curve of elongation as a function of the tension forces to which it is subjected. It is quite obvious that in the course of the operations on the thread, the latter must not be subjected to forces which tend to annul 20 the desired effect. None of the operations, especially the drying, may be carried out under tension.

A certain number of patents describe the 25 utilization of the swelling of the cellulose acetate for the purpose of facilitating the dyeing or the loading or for obtaining matt or woolly effects. But none of them has utilized the physical modification, produced in the thread of cellulose acetate by its swelling, for the purpose of rendering possible the very great twisting which is indispensable for obtaining the effect of crepe.

To this end, the essential subject matter 35 of the present application therefore consists in the utilization of this physical modification, which is made in the threads of cellulose acetate and which is preserved after the swelling agent has been removed and the threads have been dried and taken up their 40 normal content of moisture, for the purpose of imparting to these threads the high degree of twist that the authors have found to be necessary for obtaining the effects called "crepe" in the fabrics.

45 According to the invention, a swelling bath is prepared such that the thread of cellulose acetate which is immersed therein undergoes, after drying, a shrinkage of about 10 to 15%, this shrinkage being due to the 50 action of the swelling agent alone or to the combined action of the swelling agent and a colloid. The greater the shrinkage, the easier will it be to give the thread a high degree of twist but it will also be harder to obtain 55 this shrinkage without decreasing the mechanical properties of the thread. On the other hand, the smaller the shrinkage, the harder it will be to twist the thread without diminishing its mechanical properties. 60 There can be used as swelling agents all substances or mixtures of substances which are volatile or dissolved in a volatile solvent and which are capable of giving a thread of cellulose acetate immersed therein an increase of volume of at least 40 to 50%, for 65

example, sufficiently concentrated aqueous solutions of alcohol or of organic acids, aqueous solutions of certain salts as sulphocyanides, methyl alcohol, benzine, or mixtures of these bodies, on condition that these mixtures are not solvents of cellulose acetate or that, on evaporation of the more volatile part of the mixture, a solvent of cellulose acetate does not remain on the thread, unless it can be removed by a suitable washing 75 while preserving the physical modification made by the thread.

As colloids, there may be used substances such as gelatine, vegetable gums etc. and, in general, all substances that are soluble 80 in the above mentioned liquids and are capable of increasing the shrinkage imparted to the thread of cellulose acetate by the swelling agent.

Moreover, the conditions of temperature, 85 of duration of immersion, of concentration of the swelling agent and of the colloid may vary in accordance with the nature of the thread employed (titre, size of the fibres, origin), of the swelling agent and of the 90 colloid. The threads of cellulose acetate thus subjected to the action of the swelling agent are then dried or washed with a suitable liquid according to whether it is more convenient to employ drying or washing for 95 the purpose of removing the swelling agent. The latter having been removed, the dried threads, which preserve only their normal moisture content, can practically stand high 100 degrees of twist, for example 2900 to 3000 turns or more per metre for a thread with a titre of 100 deniers. The weaving of such hard twisted threads does not require any 105 special precaution; they may be used alone or mixed with any other natural or artificial textiles, and the fabrics obtained after the usual treatments of degumming and dyeing present the characteristic properties of crepes—i. e., appearance, feel, firmness and 110 elasticity.

There may be added to the swelling bath any lubricating product that can facilitate the manipulations of the thread.

*Example I.*—5 litres of ethyl alcohol are added to a bath containing 200 grams of gelatine dissolved in 5 litres of water. Cellulose acetate of 100 deniers is immersed therein at 45° C. After squeezing out and drying, the threads are given a twist of 3000 turns per metre, some being twisted to the left and others to the right. These threads are used for weaving at 27 picks per centimetre a warp of 45 threads per centimetre of cellulose acetate of 75 deniers, for example by two picks being twisted to the right and two picks being twisted to the left, the warp being run as in the case of taffeta, and there is thus obtained a fabric presenting, after 120 scouring and dyeing, a shrinkage of about 125 15 to 20% in the direction of the weft and of 130

10% in the direction of the warp, and having the characteristic qualities of a good fabric called "crêpe de Chine", an article that has never hitherto been really obtained by using 5 solely threads of cellulose acetate.

*Example II.*—Threads of cellulose acetate with a titre of 100 deniers are immersed for 15 minutes in a swelling bath consisting of an aqueous solution of nitric acid containing 10 32% of  $HNO_3$  and kept at a temperature of 15° C. These threads are then washed with water until they no longer have an acid reaction. They are then dried and given a twist of 2900 turns per metre, some being 15 turned to the left and others to the right. These threads are used for weaving at 27 picks per centimetre a warp of 45 threads per centimetre of cellulose acetate of 75 deniers, for example by two picks being twisted to 20 the right and two picks being twisted to the left, the warp being run as in the case of taffeta, and there is thus obtained a fabric presenting, after scouring and dyeing, a shrinkage of about 15 to 20% in the direction 25 of the weft and of 10% in the direction of the warp, and having the characteristic qualities of a good fabric called "crêpe de Chine".

*Example III.*—Threads of cellulose acetate are immersed for 10 minutes in a swelling liquid consisting of a mixture of carbon tetrachloride and chloroform in the volumetric proportions of one part of carbon tetrachloride to three parts of chloroform and at 30 a temperature of 15 to 17° C., after which these threads are reduced by drying in a current of air at the ordinary temperature and, after taking up moisture, they are used as indicated in one of the two preceding examples.

40 What I claim and desire to secure by Letters Patent of the United States is:—

1. Process for the treatment of threads of cellulose acetate for use in the manufacture of fabrics with crepe effect consisting in subjecting the threads before twisting to a preliminary shrinkage by first subjecting them to the action of a swelling agent and then eliminating said swelling agent and subsequently subjecting the shrunk threads to a twisting action of the order of 2800 to 3000 turns per metre for a thread of 100 deniers.

45 2. Process for the treatment of threads of cellulose acetate for use in the manufacture of fabrics with crepe effect consisting in effecting a preliminary shrinkage in length of the untwisted threads of about 10 to 15% by first subjecting them to a swelling agent to increase their volume by at least 40% and 50 then eliminating the swelling agent, and subsequently subjecting the shrunk threads to a twisting action of the order of 2800 to 3000 turns per metre for a thread of 100 deniers.

55 3. In the manufacture of crepe effect fabrics from cellulose acetate threads the

process consisting in performing the following steps in sequence:—

(1) Effecting a permanent physical alteration of the threads consisting principally in a reduction in length by approximately 70 10% to 15%, by subjecting the threads to a swelling agent to increase their volume by 40% to 50% and then eliminating the swelling agent.

(2) Subjecting the thus treated threads 75 to a twisting action of the order of 2800 to 3000 turns per metre for a thread of 100 deniers.

In witness whereof I affix my signature.

CLAUDE CLEMENCON. 80

85

90

95

100

105

110

115

120

125